

# UNITED STATES PATENT OFFICE.

CALVIN VOS, OF NEW YORK, N. Y.

## ALLOY.

1,382,147.

Specification of Letters Patent. Patented June 21, 1921.

No Drawing.

Application filed September 4, 1920. Serial No. 408,150.

To all whom it may concern:

Be it known that I, CALVIN Vos, a citizen of the United States, residing at New York city, in the county of New York and State 5 of New York, have invented certain new and useful Improvements in Alloys, of which the following is a specification.

This invention relates to an improvement in alloys.

10 The prime object of the invention is to produce an alloy in which exist degasifying and deoxidizing properties, in addition to which it will act as a medium for introducing into steel, and the ferrous groups of 15 metals, small quantities of zirconium in a fully reduced condition, thereby preventing hard spots so prevalent when zirconium is added by many other well known methods.

20 The combination of ingredients herein- 25 after described possesses properties superior to aluminum and other degasifying agents ordinarily employed, and the claim is made that it constitutes one of the few means of entirely eliminating the last vestige of oxids, gases, etc., remaining in the steel after the addition of ferro-silicon.

25 The above mentioned objects, and such other objects as may appear from the ensuing description are attained by the use of 30 my improved alloy possessing the combined composition of metals hereinafter set forth and particularly pointed out in the claims appended hereto.

35 My improved alloy consists of aluminum within the limits of from 90 to 95 per cent.; magnesium within the limits of from 2 to 10 per cent.; sodium fluorid within the limits of from 0.01 to 5 per cent.; zirconium within the limits of from 0.01 to 6 per cent.; 40 and ferro-silicon within the limits of from 0.02 to 3 per cent.

In the manufacture of the alloy, my method of procedure is as follows:

I first melt the aluminum in any suitable, 45 desirable, or convenient container, then apply heat to raise the temperature of the aluminum sufficiently to reduce it to a molten mass, then I introduce the sodium fluorid, 50 constantly stirring and agitating the whole mass gently. I then add the zirconium and the ferro-silicon in a similar manner. After 55 the aluminum, sodium fluorid, zirconium and ferro-silicon shall have been thoroughly melted and mixed together, I then add the magnesium, so that when all of the metals herein referred to are thoroughly melted and

mixed by constant gentle stirring, the alloy produced is admirably adapted for use in degasifying and deoxidizing steel and the ferrous groups of metals, thereby increasing 60 the density and eliminating the tendency of the formation of flaws in the castings obtained from said metals.

The improved alloy constituting my invention consists of an excess of aluminum 65 and magnesium properly mixed with smaller proportions of sodium fluorid, zirconium and ferro-silicon; these combined ingredients being suitably mixed and added at the proper time constitutes the means by which 70 an improved product is obtained, and which thoroughly eliminates from the steel all oxids, gases, etc., thus creating a more dense and homogeneous product, and by the use of small quantities of zirconium in a fully 75 reduced condition the formation of hard spots, usually prevalent when zirconium is added by other methods, is thereby avoided.

It will be understood that when all of the metals have been properly mixed and reduced to a molten mass, the constant gentle stirring will cause such gases as may be contained in the molten metal to escape therefrom, thereby insuring a more dense and homogeneous product.

80 By means of the ingredients and my method hereinbefore referred to, an improved alloy is obtained which is possessed of unusual tensile strength and density, and which is especially desirable in the manufacture 85 of structural work where it is of the utmost importance that such work should possess flawless qualities and the maximum of strength.

Having thus described my invention, what 95 I claim and desire to secure by Letters Patent is:—

1. An alloy possessing degasifying and deoxidizing properties consisting of a major quantity of aluminum, a minor quantity of 100 magnesium, ferro-silicon and zirconium in relatively small proportions.

2. An alloy possessing degasifying and deoxidizing properties consisting of aluminum, magnesium, ferro-silicon, and zirconium, the aluminum being approximately 105 from 90 to 95 per cent.; the magnesium from 2 to 10 per cent.; the ferro-silicon from 0.02 to 3 per cent. and the zirconium from 0.01 to 6 per cent.

CALVIN VOS